

Feb. 16, 1937.

R. E. FRICKEY

2,070,890

## RAIL JOINT AND METHOD

Filed May 28, 1934

**FIG\_1**



FIG. 2



**FIG. 3.**



FIG. 4.



FIG. 6.



FIG. 5.



FIG. 7

— INVENTOR  
Royal E. Frickey  
BY Paul D. Fehr  
ATTORNEY

## UNITED STATES PATENT OFFICE

2,070,890

## RAIL JOINT AND METHOD

Royal E. Frickey, San Francisco, Calif., assignor  
to Welding Service, Inc., San Francisco, Calif.,  
a corporation of California

Application May 28, 1934, Serial No. 727,929

9 Claims. (Cl. 238—148)

This invention relates generally to the construction of rail sections for use in conjunction with railroad tracks, to track joints which are commonly made between adjacent ends of rail sections, and to rail hardening methods applicable to the same.

In the past it has been found that rail joints are subject to rapid deterioration due to severe pounding upon the rail ends by rolling stock. Such pounding causes a battering and flow of metal at the upper edges of the rail ends, which, together with relative up and down movements, causes a chipping away of metal. Such detrimental battering can be materially minimized if the upper surfaces of the rail sections at the joints are hardened to a material degree, as by heating followed by chilling.

As hardening operations of the above character have been carried out in the past, the hardened area has been extended the full width of the rail ball, under the assumption that such an area is necessary or desirable in order to most effectively prolong the life of the joint. I have found that there is a serious disadvantage to such practice. When a rail is in use there is a tendency for wear to occur along the inner side of the rail ball, due to engagement with the wheel flanges, such wear being particularly pronounced on curves in the track. A hardened layer of metal at a joint, extending to the inner side of the rail ball, will resist such wear more effectively than the remainder of the rail ball, with the result that wear will not occur evenly. The consequence of such uneven wear will be apparent; as the unevenness becomes more pronounced, jolts will be imparted to the rolling stock, severe lateral forces will be imparted to the joint, and the desired smoothness of operation of the rolling stock over the track will be lost. After such uneven wear has occurred to a detrimental degree, the only remedy is to lay new rails or to grind off the protruding metal where hardened surfaces have resisted wear.

It is an object of the present invention to provide a rail construction and joint therefor whereby a relatively hard layer of metal will resist serious battering of the rail ends, without, however, causing uneven wear on the inner side of the rail ball. A further object of the invention is to provide a method for the treatment of rail ends, which will afford hardened areas for the joints substantially in accordance with the present invention.

Referring to the drawing:

Fig. 1 is a side elevational view illustrating a

conventional rail joint of the type with which my invention may be employed.

Fig. 2 is a plan view of the joint shown in Fig. 1, with the joint bars removed, indicating hardened areas applied in accordance with the present invention.

Fig. 3 is a cross-sectional detail taken along the line 3—3 of Fig. 2.

Fig. 4 is a cross-sectional detail taken along the line 4—4 of Fig. 2.

Fig. 5 is a plan view of a rail joint indicating the manner of heating which I prefer to employ, preparatory to chilling to effect hardening.

Fig. 6 is a view similar to Fig. 5, indicating chilling or quenching apparatus in position over the heated areas.

Fig. 7 is a side elevational view of the chilling apparatus applied to a rail joint.

Referring first to Fig. 1, the conventional rail joint illustrated therein consists of a pair of rail sections 10, secured together by joint bars 11. Each rail section is of conventional construction, consisting of a ball portion 12, bottom flanges 13, and a vertical connecting web 14.

Referring now to Figs. 2 to 4 inclusive, in carrying out my invention the upper surfaces of the adjacent rail ends are provided with hardened areas 16. Each area is in effect a hardened layer of metal which, although in thickness it constitutes a minor portion of the depth of the rail ball, is of sufficient depth to effectively minimize battering of the upper edges of the rail ends by pounding from rolling stock. These hardened rail areas need not extend for a great distance longitudinally of the rail from the center of the joint; in practice, a length of from two to three inches from the end of the rail has been found to be sufficient. In width, the area is so dimensioned that its longitudinal marginal edges 17 terminate short of the vertical side 18 of the ball. As an example of actual practice, the marginal longitudinal edges 17 of the hardened area may be spaced a distance of, say one-half inch from the vertical sides 18 in a 130 lb. rail.

In addition to affording the hardened areas, it is generally desirable to trim off or slot the adjacent rail ends, by suitable cutting or grinding operation. Thus, in Figs. 1 and 2 the upper edges of the ends of the rail sections are beveled to afford a slot, as indicated at 19, and the extension of this slot from the hardened areas 16 to the inner side of the rail is of increasing width and depth. Likewise, the inner side of the joint is

provided with a relatively wide and deep slot 20, which joins the inner end of slot 19.

As has been previously explained, the inside of the rail ball, particularly on track curves, is subject to considerable wear due to engagement with the flanges of wheels. For example, referring to Fig. 3, one side of the ball may be worn away to a contour indicated by the dotted line 21. Similar wear is indicated by the dotted line 22 in Fig. 2. It is evident from an inspection of both Figs. 2 and 3 that the hardened area or layer 16 cannot in any way interfere with such wear. This is for the reason that the sides of the rail ball adjacent the marginal edges of the hardened areas 16 are not hardened, and therefore they wear away at the same rate as the remainder of the rail. It is also evident, as has been previously explained, that if the areas 16 were extended to the side surfaces 18 of the ball, and if such extensions of area 16 were of the same order of hardness, such wear would not occur evenly throughout the length of the rail and laterally protruding hardened surfaces would be formed at the joint.

Wear upon the inner side of the rail ball, such as described above, is also accompanied by a pounding upon the inner edges of the rail ends, with the result that there is a tendency for metal flow to occur, particularly since the metal at this point is not hardened. The relatively wide slot 20, together with the widening of slot 19 as it merges with slot 20, mitigates such tendency toward metal flow, and avoids detrimental effects if metal flow does occur to a material degree.

Assuming that the rail sections are to remain in a permanent position, there can be no objection to extending the hardened area to the outer side of the rail ball, since wear of the character to which I have referred is confined to the inner side of the rail ball. However, the arrangement which I have described, in which the hardened areas terminate short of both sides of the rail ball, is desirable in that it permits the rails to be reversed after one side of the ball has been worn to a serious degree. Likewise, such construction permits reversible laying of rail sections, where the sections are treated to provide the hardened areas before being laid.

Various methods can be utilized to provide hardened areas in accordance with my invention. However, it has been found desirable to utilize the general method disclosed in copending application Serial No. 660,544, in which a confined and limited area of the upper surface of the rail is heated by means of a rapidly moving electric arc, followed by chilling by forming a confined pool of liquid upon the heated area. Proper limiting of the extent of the hardened areas can be effected by definitely limiting the extent of heating, or by limiting the area of chilling, or by both. Thus, as shown in Fig. 5, I have indicated heating by rapidly traversing an electric arc over an area commensurate with the desired extent of the hardened area 16. Following heating to a proper degree, open-bottomed boxes 23 are positioned on top of the rail, and a suitable chilling liquid, such as oil, is introduced through pipes 24. The lower edges of the boxes are provided with gaskets or like means for forming a seal with the upper surface of the rail, so that confined pools of liquid are formed upon the heated area. Pipes 26 are indicated for removal of the liquid for re-use. The time period of chilling is controlled to secure the desired degree of hardness, and following the chilling operation

heat may be permitted to flow back into the hardened areas for tempering or drawing.

I claim:

1. In a rail joint having aligned rail sections connected by joint bars or like means, the rail sections having ball, web and flange portions, a hardened layer of metal in the upper surface of the ball of each section, the area of extent of each layer being for a substantial distance along the length of the rail from the adjacent rail ends and for a substantial distance laterally of the rail ball, to minimize battering of the rail ends, the marginal edges of the layers corresponding to the inside of the joint terminating short of the inner face of the rail ball, whereby the inner face of the rail ball may wear away evenly, the upper and inner edges of the rail ends being beveled to afford a lateral slot which extends across the joint and joins an upright slot on the inner side of the rail ball, the inner slot 20 being relatively wider and deeper than the intermediate part of the lateral slot.

2. In a method of the character described for hardening rail ends, heating and chilling an upper layer of metal at the end of a rail section to effect hardening of the same, and causing the hardening to be substantially limited to an upper area of the rail ball which terminates short of the inner side of the rail ball.

3. In a method of the character described for hardening rail ends, heating and chilling an upper layer of metal at the end of a rail section to effect hardening of the same, and causing the hardening to be substantially limited to an upper area of the rail ball which terminates short of both the inner and outer sides of the rail ball.

4. In a railroad rail section having an ungrooved ball, and also having web and flange portions, a hardened layer of metal in the upper surface of the ball, the area of extent of said layer being for a substantial distance along the length of the rail section from one end thereof and for a substantial distance laterally of the rail ball, to minimize battering of the rail end, the hardened layer being of substantial depth, that longitudinal marginal edge of the layer, corresponding to the inside of the rail section when laid in a track, terminating short of the inner surface of the rail ball, whereby the inner face of the ball which engages the wheel flanges may wear away evenly.

5. In a railroad rail section having an ungrooved ball, and also having web and flange portions, a localized layer of metal in the upper surface of the ball, which is substantially harder than the remainder of the rail metal, said layer having substantially the same essential ingredients as the remainder of the rail metal, the areas of extent of said layer being for a substantial distance along the length of the rail section from one end thereof and for a substantial distance laterally of the rail ball, to minimize battering of the rail end, the layer being of substantial depth, the longitudinal marginal edges of the layer terminating short of both sides of the rail ball.

6. In a rail joint having aligned rail sections connected by joint bars or like means, the rail sections having an ungrooved ball, and also having web and flange portions, a localized layer of metal in the upper surface of the ball of each rail section which is substantially harder than the remainder of the rail metal, the hardened layer being of substantial depth, the area of extent of each layer being for a substantial distance along the length of the rail from the adjacent rail ends.

for a substantial distance laterally of the rail ball, to minimize battering of the rail ends at the joint, the marginal edges of the layers corresponding to the inside of the joint, terminating short of the inner faces of the ball, whereby the inner face of the rail ball may wear away evenly.

7. In a rail joint having aligned rail sections connected by joint bars or like means, the rail sections having an ungrooved ball, and also having web and flange portions, a localized hardened layer of metal in the upper surface of the rail ball of each section, the hardened layer being of substantial depth, the area of extent of each layer being for a substantial distance along the length of the rail from the adjacent rail ends and for a substantial distance laterally of the rail ball, to minimize battering of the rail ends, the longitudinal marginal edges of the layers terminating short of both the inner and outer edges of the rail ball.

8. In a method of the character described for hardening rail ends, heating an upper layer of metal at the end of a rail section, and then effecting localized contact of the heated metal with a chilling liquid to harden the same, contact of the chilling liquid being limited to an area which terminates short of the inner side of the rail ball.

9. In a railroad rail section having an ungrooved ball, and also having web and flange portions, a hardened layer of metal of substantial depth in the upper face of the ball at one end of the rail section, whereby the tip of the rail section resists the pounding of rolling stock, said layer being substantially localized with respect to the inner face of the rail ball whereby the inner face of the rail ball in the proximity of said area can wear away to a substantial extent at substantially the same rate as portions of the inner face remote from said hardened area.

ROYAL E. FRICKEY. 20